

## UNITED STATES PATENT OFFICE

2,097,024

PRODUCTION OF A PROTECTIVE LAYER ON  
IRON

Walter Enders, Solingen-Ohligs, Germany

No Drawing. Application October 26, 1936, Serial  
No. 107,732. In Germany November 5, 1935

5 Claims. (Cl. 148—14)

A great variety of processes are known for the production of a protective layer on iron (steel), also by way of cementation, that is by heating the iron surrounded by a powder (cementation powder) in a closed container. In this cementation powder aluminium powder usually plays the chief part.

According to the present invention a particularly heat-resisting protective layer is produced by a cementation which also makes use of aluminium powder, but in combination with powdered silicon and without any non-metallic addition. Either a mixture of the two powders or preferably a powdered aluminium-silicon alloy is used. The silicon content amounts to from 15 to 80%, preferably about 30 to 40%. The proportion of aluminium and silicon must at any rate be such that besides the aluminium the silicon is alloyed into the iron in a quantity which substantially affects the heat resistance.

A protective layer on iron (steel), produced in accordance with the invention, has proved to be particularly resistant to high temperatures (not liable to form scale), but is also capable of withstanding corrosion and wear.

For the rest the process with aluminium and silicon is carried out in the known manner. The powder consisting of aluminium and silicon is placed with the article to be cemented in a closed container and brought to a high temperature, in the case under discussion to about 1000°.

The process has been tried out with aluminium and silicon, but besides the silicon another metal-

loid or metal may be added, for instance chromium, manganese, titanium or the like. An addition of metal oxides or metal salts or any other non-metallic addition is however unnecessary and may even have a disturbing effect, as for instance the addition of binders.

What I claim is:

1. A process for the production of a protective layer on iron or steel, consisting in surrounding the iron with a powdered material consisting of 10 aluminium and silicon in a closed vessel and applying heat thereto, whereby the silicon as well as the aluminium become alloyed with the iron to increase the heat resistance thereof.

2. A process for the production of a protective layer on iron or steel, consisting in surrounding the iron with a mixture of powdered aluminium and powdered silicon in a closed vessel, and applying heat thereto, whereby the silicon as well as the aluminium become alloyed with the iron to increase the heat resistance thereof.

3. A process as claimed in claim 2 wherein the silicon content of the mixture is 30 to 40%.

4. A process for the production of a protective layer on iron or steel consisting in surrounding the iron with an aluminium silicon alloy in powdered form in a closed vessel and applying heat thereto, whereby the silicon as well as the aluminium become alloyed with the iron to increase the heat resistance thereof.

5. A process as claimed in claim 4 wherein the silicon content of the alloy is 30 to 40%.

WALTER ENDERS.